

## UNITED STATES PATENT OFFICE

2,433,632

FIBROUS SHEET MATERIAL FOR THE  
ELECTROLYTIC FORMATION OF AZO  
DYE IMAGE RECORDS THEREON

Myer Solomon, deceased, late of Westmont, N. J.,  
by Nellie W. Solomon, administratrix, Princeton,  
N. J., assignor to Radio Corporation of  
America, a corporation of Delaware

No Drawing. Application December 23, 1942,  
Serial No. 469,961

4 Claims. (Cl. 204—2)

1

This invention relates to the electrolytic production of azo dyes by electrolytic coupling and more particularly to an article of manufacture carrying the dye-forming constituents. In a preferred adaptation it includes such an article for the production thereon of azo dyes by electrolytic coupling in connection with the art of facsimile recording. The fundamentals of the present disclosure are set forth in the copending application, Serial No. 178,743, now U. S. P. 2,306,471, included herein by reference, of which earlier application the present application is a continuation-in-part.

The present invention may be generally stated to embrace features pertaining to the electrolytic coupling of a diazonium compound with the production of an azo dye. In a desirable embodiment involving the application of the invention, the dye is produced in situ on a supporting material adapted to receive the same. Where the current which actuates the electrolytic coupling is dependent upon electric impulses from a transmitting source, such as a scanning station for the transmission of printed matter, a picture, etc., the electrolytic coupling and dye formation serve in the capacity of a facsimile recorder to form images or reproductions determined by the characteristics of the transmitted electrical impulses from the scanning station. The following description is primarily directed to this sphere of the invention described in the aforesaid copending application, Serial No. 178,743.

It is an object of the invention to overcome the difficulties and limitations of the prior art procedures noted hereinabove.

It is another object of the present invention to obtain azo dyes by the effect of an electric current on mixtures or solutions containing a diazonium compound and a coupling compound.

An additional object of the invention is to produce azo dyes by treatment of mixtures or solutions of reagents adapted to form a diazonium compound and electrolytically coupling this compound with a coupling reagent.

It is a further object to provide mixtures or solutions containing a diazonium compound and a coupling compound which are adapted to electrolytically react for the purpose of producing azo dyes.

Still another object is a supporting material

2

or carrier impregnated with a diazonium compound and a coupling compound under conditions which will preclude coupling and azo dye formation until the influences engendered by an electric current actuates such coupling and azo dye formation.

An important object of the invention is to obtain articles of manufacture adapted for facsimile recording in the form of a carrier or supporting material treated with a diazonium compound and a coupling compound under conditions which will preclude azo dye formation until coupling is actuated electrolytically by electric impulses from a transmitting source which correspond with the visual characteristics of the object at the transmitting source.

Other objects, features and advantages of the invention will be apparent from the following consideration and description thereof.

In the present invention, wherein facsimile recording is contemplated, it is proposed to produce the picture or printed matter on the recording surface in the form of an azo dye, the amount of such dye deposited being a function of the amount of current caused to flow through the recording surface, which is conveniently a paper sheet or web. When the image is formed in the nature of an azo dye electrolytically produced, the pressure of the printer bar is maintained constant and the amount of current which is passed through increments of the paper varies in accordance with the light and dark portions present on the object, the likeness of which is being reproduced, such as a picture or printed matter, by scanning at the facsimile transmitter. When the dyes are thus formed electrolytically, varying halftone shades are obtained as a result of the variation in the amount of current caused to flow through the recording paper.

The principle of operation of the present invention resides broadly in the fact that a diazonium compound and a coupling compound which is adapted to react in alkaline, neutral or mildly acid solution, may be combined to form an azo dye when subjected to electrolytic treatment. Thus, electrolytic coupling of diazonium compounds may be attained when a mixture of coupling reagent and diazonium compound reacts in an alkaline solution to form an azo dye, the coupling component being of the type which will

couple in an alkaline medium; under these conditions, the dye is produced at the alkaline or negative electrode, usually designated as the cathode. Similarly, where the coupling compound is of the type which reacts with the diazonium compound in an acid medium, coupling will take place under appropriate conditions. The distinction between alkaline reacting coupling reagents and acid reacting coupling reagents is considered in some detail hereinbelow.

Applying this principle and theory to the present invention, where the diazonium compound and the coupling component are maintained in an acid medium, and the coupling compound is of the type which will react in alkaline medium, formation of azo dye is effectively prevented until such time as the solution is subjected to an electric current. Under the latter conditions, alkalinity is established at the cathode, thereby forming a zone of coupling reaction which is substantially instantaneous in character. Differently stated, the electrolytic coupling, in accordance with the present invention, is predicated on the conditions of control for retaining the diazonium compound and the coupling compound in a medium which will preclude their interaction until such time as a current is passed through the electrolytic cell wherein coupling is contemplated. This control depends upon the fact that the diazonium compound and the coupling agent which functions in alkaline medium will not react in an acid medium, but will couple in an alkaline zone, even though such zone may be comparatively limited in its scope, and, in fact, occurs in the immediate vicinity of the cathode.

For facsimile recording, the recording surface may be rendered wet by a mildly acid solution containing diazonium and alkaline reacting coupling compounds, and is then passed through the facsimile receiving or recording apparatus in such a manner that electric current causes dye formation on the receiving surface corresponding to the transmitted picture or printed matter, as a result of electrical impulses received from the facsimile transmitting device at which point the picture or printed matter is positioned.

A solution is prepared containing essentially the following ingredients:

I. A neutral electrolyte, such as sodium or potassium chloride or sulphate. This serves to facilitate the flow of electric current through the paper.

II. A diazonium salt, desirably one sensitive to light.

III. A coupling compound, desirably of the aromatic hydroxy type, coupling essentially under alkaline conditions.

IV. A small amount of an acid, to maintain the acidity of the solution and thus prevent premature coupling.

V. Water or other solvent in which the electrolyte ionizes.

In addition to the ingredients above indicated, the solution may also contain perfecting ingredients pursuant to the particular function to be attained or characteristic to be provided. Among such perfecting ingredients may be listed: (1) "coupling inhibitors," as semicarbazide or hydroxylamine, which aids acidity in preventing premature coupling, (2) reducing agents, as sulphites, hydrosulphites, thiosulphates, hydroquinone, glucose, tartrates, oxalates, stannous chloride, etc., which prevent the gradual darkening

5  
10

of the background, (3) salts of copper, iron, chromium, aluminum or other metals, which act as mordants or otherwise affect the color of the dyes or the light sensitivity of the diazonium salt, or (4) reagents adapted to effect background permanence, color intensity, and threshold value.

For simplifying the consideration of the invention, the discussion will primarily be directed to the case where the coupling compound is of the character which reacts in an alkaline medium, especially since such coupling compounds have manifested generally improved results over that attainable in the case of operating under conditions where an acid reacting coupler may be utilized. Briefly indicated, the reaction involves the azo dye formation at the negative or alkaline electrode; i. e., the cathode, the electric current creating an alkaline condition which persists long enough for the diazonium and the coupling compound or compounds to combine with each other.

Thus, if the invention is used in facsimile recording, once having electrolytically coupled the diazonium salt by electric impulses emanating from a transmitting source at which an object or picture is subjected to scanning, and thereby obtaining a facsimile on the recording sheet corresponding with the object or picture, in the form of an azo dye, the unreacted diazonium salt may then be removed from the recording sheet by decomposing said salt through the action of light or heat. Alternatively, washing may be resorted to for accomplishing the removal of unreacted reagents.

The following is a generalized example of the ingredients which may be utilized to form a solution whereby a dye may be produced by electrolytic coupling. It will be noted that this example embraces within its scope and contemplation the use of caustic soda; this reagent is applicable only under extenuating circumstances which will be explained in further detail hereunder.

| Ingredients                                                                    | Gram-Molecular Weight Used | Amount Used                               |
|--------------------------------------------------------------------------------|----------------------------|-------------------------------------------|
| (I) A mine-source of Diazo-nium Salt.                                          | .033-----                  | Varies with molecular weight of amine.    |
| (II) Hydrochloric acid: Normal solution (or equivalent amount of other acids). | .08-----                   | 80 cc.                                    |
| (III) Sodium Nitrite-----                                                      | .03-----                   | 2.07 grams.                               |
| (IV) Coupling compound; hydroxy aromatic compound.                             | .010 to 0.15-----          | Varies with molecular weight of compound. |
| (V) Sodium Chloride -----                                                      | 1.0-----                   | 58.47 grams.                              |
| (VI) Ice and water to total volume of 1000 cc.                                 | -----                      |                                           |
| (VII) Sodium Hydroxide: Normal solution NaOH.                                  | .05 to .1-----             | 50 to 100 cc. Used only in special cases. |
| (VIII) Auxiliary Chemicals such as reducing agents.                            | Varying amounts-----       |                                           |

A desirable illustrative procedure of mixing the ingredients is as follows:

The source of diazonium ion, desirably a primary amine (I), may be dissolved in the acid with boiling and addition of small amounts of water as necessary. The resulting amine hydrochloride solution is then desirably cooled to approximately 0° to 8° C., preferably by adding ice. The ionizable nitrite (III), such as sodium nitrite, is dissolved in 25 to 55 cc. of water and slowly poured into the cooled solution while constantly agitating. Generally, one or more color

changes take place, accompanied by a slight effervescence, due to nitrogen gas formation. This effervescence represents a loss of diazonium compound, and it is this tendency which renders it desirable to maintain the reaction in the cold, through ice utilization. On the other hand, in some instances essentially no gas appears even at ordinary room temperatures—i. e., 20° C.—30° C. The coupling compound (IV) and the electrolyte (V) are dissolved in water either together or separately, and added to the mixture of amine, acid and nitrite, above indicated, after that mixture has been permitted to stand for a period of at least fifteen minutes.

The caustic soda (VII) is used only where the amine (I) is an amino-sulphonic or amino-carboxylic acid insoluble in the acid (II). Under such circumstances, the amine is dissolved in the alkaline solution (VII), and the acid requirements must then be increased by an amount equivalent to the alkaline reagent utilized and to provide the desired acidity. The basic amine solution is slowly poured into a mixture containing acid, nitrite, as well as the cooling expedient exemplified by ice. Auxiliary chemicals, if used, are desirably added with the coupling compound (IV).

If an amine hydrochloride, or a poly-amino compound is used as ingredient (I), the amount of hydrochloric or other acid is changed accordingly, so that when I, II and III are finally mixed

6  
diamine, a substantial number of amino sulphonic acids of benzene, naphthalene or diphenyl compounds, and some naphthol sulphonic acids. As a general matter, the presence of sulphonate groups has functioned quite favorably in the production of azo dyes, and this type of compound has been especially effective in connection with the facsimile recording sheet upon which the azo dye is to be produced in accordance with any predetermined recordation. It will be apparent that the amines may be of the mono-amino benzene, poly-amino benzene, amino-naphthalene, and amino poly-phenyl types of compounds.

15 It should be noted that among the most desirable diazonium sources are the para diamino benzenes, since their diazonium salts are quite sensitive to light, provide comparatively dark colors, and have substantially no tendency to couple in mild acid solution. Alkyl groups on one of the amino nitrogens serve to improve the depth of color, while acid (acetyl or oxalyl) groups may in some instances weaken the shade and even reveal some tendency toward premature coupling in acid solution.

20 25 Following are presented a number of amino compounds which have quite effectively functioned as sources of diazonium compounds, the latter effectively reacting electrolytically with a 30 coupling compound adapted to form azo dyes therewith in alkaline medium:

#### Amines—Sources of diazonium compounds

| Name of Amine                                                                                                                                                                                                                              |                                                                                                                                                                                                  | Color and background after exposure to light when used with phloroglucinol as a coupling compound                                                             |
|--------------------------------------------------------------------------------------------------------------------------------------------------------------------------------------------------------------------------------------------|--------------------------------------------------------------------------------------------------------------------------------------------------------------------------------------------------|---------------------------------------------------------------------------------------------------------------------------------------------------------------|
| Common Name                                                                                                                                                                                                                                | Structural Name or Formula                                                                                                                                                                       |                                                                                                                                                               |
| Metaphenylenediamine<br>2-amino-5-diethylaminotoluene                                                                                                                                                                                      | 1,3-diaminobenzene<br>1-methyl-2-amino-5-diethylaminobenzene                                                                                                                                     | Brown-yellow on white.<br>Dark brown-purple on very pale yellow.                                                                                              |
| Paraminodiethylaniline<br>Paraminodimethylaniline<br>2,5-diaminoanisole<br>2,5-diaminoanisole dihydrochloride<br>Paraphenylenediamine<br>4-aminodiphenylamine<br>4-aminodiphenylamine mono-hydrochloride<br>3-methyl-4-aminodiethylaniline | 4-amino-1-diethylaminobenzene<br>4-amino-1-dimethylaminobenzene<br>2,5-diamino-1-methoxybenzene<br>1,4-diaminobenzene<br>1-phenylamino-4-amino benzene<br>3-methyl-4-amino-1-diethylaminobenzene | Do.<br>Do.<br>Dark brown on pale tan.<br>Do.<br>Orange-brown on white.<br>Purple on white.<br>Deep purple on white.<br>Dark brown-purple on very pale yellow. |
| Chicago or 2S acid<br>Paraaminooctanilid<br>Paraaminomethylacetanilid<br>Gamma acid                                                                                                                                                        | 1-amino-2,4-disulpho-8-hydroxynaphthalene<br>4-amino-1-acetylaminobenzene<br>4-amino-1-methylacetylaminobenzene<br>2-amino-8-naphthol-6-sulphonic acid                                           | Dark purple on white.<br>Orange on orange.<br>Orange on pale yellow.<br>Do.<br>Orange-brown on orange.                                                        |
| 4,4'-diaminodiphenylmethane                                                                                                                                                                                                                |                                                                                                                                                                                                  | Dark orange on light orange.                                                                                                                                  |
| 4-amino-benzylethylaniline                                                                                                                                                                                                                 |                                                                                                                                                                                                  | Purple on white.                                                                                                                                              |
| Oxalyl paraphenylenediamine<br>4-aminodiphenylamine-2-sulphonic acid<br>1,24-acid                                                                                                                                                          | N-oxalyl-1,4-diaminobenzene<br>1-phenylamino-4-amino benzene-2-sulphonic acid<br>1-amino-2-naphthol-4-sulphonic acid                                                                             | Orange on pale orange.<br>Red on pink.<br>Deep purple on pale straw-yellow.<br>Background white when washed.                                                  |

there are .05 gram equivalent weights of acid for the .03 of sodium nitrite, in addition to the acid required to neutralize all of the amino groups present in the amino compound.

Relative to the amines within the purview of the disclosure, substantially any diazotizable amino compound will serve as a source of diazonium compound. Primarily, the amino compounds will be primary aromatic amines. Desirably, these amino substances should be acid soluble, and in addition should not be too readily susceptible to oxidation, electrolytic, or by air or in any other manner. Included among the amines which may be used are meta-phenylene

In lieu of commencing with the primary amine and the ionizable nitrite, in order to prepare the diazonium compound, stabilized diazonium compounds, illustrated by the nitrosamines, chlorostannates, or other double salts may be used, although they may require an added amount of current in connection with facsimile recording. Starting with these salts, they are merely dissolved in water which is rendered slightly acid, following which the coupling compound and any auxiliary chemicals may be supplied prior to subjecting the solution to electrolytic treatment for the purpose of forming dyes, and if desirable at a predetermined area or zone.

The quantity of coupling compound which may be used in the above generalized example will vary with the coupling strength. Usually darker colors are produced by using more than one gram-molecular equivalent of diazonium salt per gram-molecular equivalent of coupling compound, due probably to partial formation of dyes having two or three molecules of diazonium salt coupled to one molecule of the coupling compound. As previously stated, they are preferably of the type which will couple in alkaline medium, and should be soluble in mildly acid solution. In addition, they are preferably subject to the same oxidation resisting properties as indicated above in connection with the amines. Aromatic compounds with hydroxy, amino or active methylene groups ortho or para to unsubstituted positions in the ring will usually couple. Sulphonic groups have a desirable effect along the lines suggested of the amines. Generally, favorable results have been obtained in the use of resorcinol, phloroglucinol, the naphthols and their sulphonic acids, 8-hydroxy quinoline, and some amino naphthol sulphonic acids. Taken as a whole, meta polyhydroxy benzene derivatives have reacted favorably as coupling compounds. Of the naphthalenes, Chicago acid has given optimum results, although its amino group may tend to increase the darkening of the background.

Particularly notable is the fact that some amino naphthol sulphonic acids, such as gamma, H, J, S and 2S acids, may either diazotize or couple. Good results are therefore obtainable using the same compound for forming both the diazonium compound and coupling. Where amino naphthol sulphonic acids are utilized in connection with facsimile recordings, the carrier sheet should desirably be subjected to washing after electrolytic recordation in order to stabilize the sheet background by obviating any tendency toward darkening during an interval of storage.

Following are a number of couplers which have functioned quite effectively in connection with a diazonium salt present in an acid medium, when the coupling has been actuated by electrolytic means:

coupling compounds are added. This may be accomplished with facility by using a 10% excess of amine or by adding a small amount of urea to the amine-nitrite mixture before the remaining ingredients are supplied.

As above indicated, ordinary table salt may be relied upon for effective functioning as the electrolyte of the composition. It is not essential to accurately weigh the content of the electrolyte, since substantially any amount between 40 and 120 grams per liter provides practically identical recordings in most cases. In lieu of NaCl, and merely by way of illustration, other strong neutral electrolytes are NaBr, KBr, KCl, LiCl, BaCl<sub>2</sub>, CaCl<sub>2</sub>, MgCl<sub>2</sub>, K<sub>2</sub>SO<sub>4</sub>, Na<sub>2</sub>SO<sub>4</sub>, MgSO<sub>4</sub>, etc. Some dye intermediates may manifest greater solubility in potassium chloride solutions than in sodium chloride solutions; under such circumstances, the substitution is desirable. From the standpoint of preparation of sheets for facsimile recording, lithium chloride has been found to retard the paper drying time, but an equivalent and probably more effective result is obtained by the use of wetting agents. An additional electrolyte which has provided excellent recordings, while at the same time obviating the corrosive effect of nascent chlorine, has been found to be sodium sulphamate, NaOSO<sub>2</sub>NH<sub>2</sub>.

While sodium hydroxide is illustrative of a desirable embodiment of reagent for providing the desired alkaline solution in the exceptional cases above mentioned, other well known alkaline substances may be resorted to in lieu thereof, such as potassium hydroxide.

A number of auxiliary chemicals are available for the purpose of controlling such elements as background permanence, color intensity, color characteristics, threshold value, etc. In addition, these reagents may function to preserve the time during which the reagent solutions utilized will maintain their effectiveness. Coupling inhibitors, such as semi-carbazide or hydroxyl amine, combine with the coupling compound in acid solution and thus prevent or retard premature coupling, and liberate free coupling compound upon alkalization. Reducing agents

#### Coupling compounds

| Common Name          | Structural Name or Formula                    | Remarks                                                                                                                         |
|----------------------|-----------------------------------------------|---------------------------------------------------------------------------------------------------------------------------------|
| Phloroglucinol       | 1,3,5-trihydroxybenzene                       | Quite desirable results.                                                                                                        |
| Resorcinol           | 1,3-dihydroxybenzene                          | Excellent, but give lighter colors than phloroglucinol.                                                                         |
| Orcinol              | 1-methyl-3,5-dihydroxybenzene                 | Darker color and not quite as effective as phloroglucinol with respect to definition and background.                            |
| Pyrogallol           | 1,2,3-trihydroxybenzene                       | Usually gives blue recordings. Excellent when used with phloroglucinol.                                                         |
| Chicago or 2S acid   | 1-amino-8-naphthol-2,4-disulphonic acid       | Similar to Chicago Acid, with somewhat weaker colors.                                                                           |
| Chromotropic acid    | 1,8-dihydroxynaphthalene-3,6-disulphonic acid | Good colors, but background not quite as satisfactory as with phloroglucinol or resorcinol, possibly due to premature coupling. |
| Dioxy S acid         | 1,8-dihydroxynaphthalene-4-sulphonic acid     | Generally weak colors.                                                                                                          |
| H acid               | 1-amino-8-naphthol-3,6-disulphonic acid       | Better than salicylic acid, but weaker than resorcinol.                                                                         |
| 8-hydroxyquinoline   | 8-hydroxyquinoline                            |                                                                                                                                 |
| Salicylic acid       | 2-hydroxybenzoic acid                         |                                                                                                                                 |
| Beta Resorcylic acid | 2,4-dihydroxybenzoic acid                     |                                                                                                                                 |

The performance of the process particularly in connection with the diazotization of the primary amine in acid medium is not restricted to the use of sodium nitrite as the diazotizing reagent. A comparatively wide range of nitrites are available, desirably a metallic salt, the requisite being that the nitrite be appropriately ionizable. While sodium nitrite provides quite satisfactory results, the same may be attributed to potassium nitrite as well as a number of other metallic nitrites. It is desirable that no uncombined nitrite remains in solution when the

such as sulphites, hydrosulphites, thiosulphates, 65 glucose, tartrates, oxalates, formates, stannous chloride, etc., retard air oxidation, thereby aiding in preserving the background permanence of recordings which have been fixed by exposure to strong light. Salts of copper, iron, chromium, 70 aluminum, and other metals frequently serve as mordants or otherwise effect the color and fastness of the dyes, or the sensitivity to light of the diazonium salts.

While water is a most desirable vehicle for 75 the electrolytic reaction, the invention is not re-

stricted to the use of the same. Thus, various non-aqueous solvents which permit electrolytes to ionize may be substituted for all or a part of the water. The alcohols serve to enable the use of the contemplated compositions at below freezing temperatures. In addition, they serve to retard the drying of recording sheets. A desirable alcohol is illustrated by normal propyl alcohol. Similarly, the solution may be a mixture of propyl with ethylene glycol. However, vehicles which boil at comparatively low temperatures may manifest some undesirable characteristics such as rendering a recording comparatively limp and moist.

The following example indicates the use of definite reagents in the preparation of the diazonium compound as well as the coupling component used to react therewith electrolytically; in addition, a desirable procedure applicable to this example is presented:

5  
ness is obtainable, and the background maintains its improved characteristic for a substantial interval of time. The amount of water utilized during the course of the successive steps is not

10  
5 of critical significance, and within the skill of one working in the field; the element which is of significance is that the total volume will satisfy predetermined amounts.

10  
The tartaric acid in the above example functions in a dual capacity, since it provides the necessary acid as well as serving as a reducing agent tending to preserve the background color.

15  
As a simplifying expedient in the handling and storage of the reagents used, they may be subjected to premixing or packaging in the form of dry powders which the ultimate user will merely dissolve in water or any other satisfactory vehicle at the time that the formation of the diazonium salt and electrolytic treatment is to be performed.

20  
20 For this purpose, solid acids are available, as

*Example*

| No.       | Ingredients, Name                             | Formula                                                                             | Use                                          | Grams used per liter |
|-----------|-----------------------------------------------|-------------------------------------------------------------------------------------|----------------------------------------------|----------------------|
| I.....    | p-Aminodiethylaniline monohydrochloride.....  |   |                                              | 4.41                 |
| II.....   | p-Aminodimethylaniline monohydrochloride..... |  | Amines—sources of diazonium compounds.....   | 1.90                 |
| III.....  | Tartaric acid.....                            | (CHOHCOOH) <sub>2</sub> .H <sub>2</sub> O.....                                      | Acid. Source of hydrogen ion; reducing agent | 6.22                 |
| IV.....   | Sodium Nitrite.....                           | NaNO <sub>2</sub> .....                                                             | To whiten background.                        | 2.07                 |
| V.....    | Phloroglucinol.....                           |  | To diazotize I and II.....                   | .042                 |
| VI.....   | Chicago or 2S acid.....                       |  | Coupling Compound.....                       | 2.39                 |
| VII.....  | Common Salt.....                              | NaCl.....                                                                           | do.....                                      |                      |
| VIII..... | Water.....                                    |                                                                                     | Electrolyte                                  | 58.47                |
|           |                                               |                                                                                     | To total volume of one liter.                |                      |

I, II and III are dissolved in cold water, IV is added and the mixture allowed to stand at least 15 minutes, during which time V and VI are dissolved in water, warming if necessary, and VII is added to the solution of V and VI with stirring until dissolved. The two solutions are mixed and water added to produce the desired volume, such as one liter. In summer, it is necessary to cool the water (preferably by adding ice) in which I, II and III are dissolved.

The solution give purplish-blue, almost black recordings on a yellowish green background. Exposure for one-half minute to a carbon arc light, or three to five minutes to direct sunlight bleaches the background until it is almost white. On standing for several weeks, the white background thus obtained becomes pale grey-brown. If the freshly recorded copy is washed with water, with or without first exposing it to strong light, an improvement in immediate background white-

60  
illustrated by tartaric, citric, oxalic, succinic, maleic, sodium acid sulphate, etc. By way of illustration, the amine, the acid, the nitrite, and a part of the electrolyte may be packaged in

60  
60 layers, each layer being separated by a layer of the electrolyte salt, such as NaCl, wads of cotton or other repellent material being applied to the top of the package or container for retaining the assembled layers in position. The remaining

65  
65 solids, such as the coupling compound and the balance requirement of the salt, as well as the auxiliary chemical, if used, will constitute a second package. In the event that the use of caustic soda is contemplated, three packages are desirable, one containing the amine and the caustic soda, the second including the solid acid and the nitrite, and the third embracing the coupling compound as well as the auxiliary chemicals; the electrolyte may be included in either of the

11

three packages or distributed amongst all of them.

When packaged in this manner, the compounds are storable for comparatively long intervals of time. As previously indicated, when performance of the process is contemplated, it is merely necessary to dissolve the respective packages in an appropriate vehicle of predetermined volume. As for the solutions, they have been stored for as much as a week without any material effect upon their strength. It is desirable to store these solutions in the darkness. Where separate solutions of diazonium salts and coupling compounds are provided, the storable time interval is very materially extended, and such solutions have been retained for many months without diminishing their effective characteristics.

The carrier on which the azo dyes are formed may be of any fibrous material, such as cloth, films, and cellulosic material generally utilized in the production of sheets, including those made from regenerated cellulose and the like. The use of paper, desirably that of rag origin, has been found particularly satisfactory for purposes of facsimile recording, and will be primarily referred to herein as illustrative of the carrier material or sheet utilized. It will be noted that the formation of the dye in situ on the fabric or paper surface comprises a desirable embodiment of the facsimile recording procedure. However, it is similarly within the scope of the present disclosure to apply the dye to yarn, and fibers per se in order to provide these materials with appropriate coloring for any intended usage.

A convenient, expedient method for treating the paper or its equivalent prior to facsimile recording involves the passage of the sheet through a bath of solution containing the reagents which essentially comprise an acid solution of a diazonium salt and a coupling compound, together with any perfecting ingredients particularly a reducing agent which may be supplied for a predetermined purpose. After the excess fluid has been removed from the paper, which is nevertheless in moist condition, it may be passed through a bar-helix type of recorder, with the bar and helix respectively serving as cathode and anode. However, many modifications of this procedure may be resorted to, both with respect to the details of apparatus and the preparation or condition of the carrier sheet.

Thus, the chemicals essential to the electrolytic coupling may be applied in more than one operation, and expediently the chemical solution may be applied to the carrier surface by means of a roller or wick. Alternatively, the carrier may be supplied with the reagents and then stored in a dry condition for usage, preferably being protected from light exposure and avoiding any lengthy storage period. When the sheet is to be passed through the recording device, it may be previously moistened by resort to a roller or wick, the moistening vehicle being either water or any other solution which will permit appropriate ionization of the substances involved in the electrolytic coupling reaction.

In lieu of the sheet immersion immediately prior to its passage through the recording mechanism, and the preparation of a dry sheet to be moistened at the time of its application to the recording device, the sheet may be stored in a moist condition, and used directly in this condition when recording is to be carried out. However, this manner of retaining the recording sheet is subject to considerable storage difficulty as a

12

result of the tendency of the diazonium compound to decompose, as well as the possibility of darkening of the background during the moist storage interval. The inherent characteristics of the paper, i. e., its inherent acidity, may be effectively taken advantage of in the matter of appropriately storing the recording sheet; in other words, where the paper manifests a distinct acidity, the impregnation or surfacing of the same with the diazonium compound and the coupling reagent will show a distinctly greater stability, for the above considered reason that an acid medium tends to prevent premature dye formation, until such time as the reagents are subjected to the passage of an electric current.

An additional effective manner of applying the chemicals to the sheet involves the production of the diazonium salt on the paper or carrier by successive applications of amine and nitrite, whereby otherwise insoluble diazonium compounds may be used.

The electrolytic coupling may be accomplished in the form of different recordings on each side of a given sheet which has been appropriately prepared; this effect is obtainable by alternate line scanning with automatic current reversal between each alternate line, preferably utilizing non-oxidizing electrodes, such as platinum. It will be noted that in the case of the bar- and helix-recording, the recording on the bar side is generally preferable.

As a general rule, electrolytic coupling may be accomplished without any particular regard for the metallic characteristics of the recording cathode; the greatest electrode wear is manifested at the positive helix electrode where a bar- and helix-type of recorder is used. Iron, copper, nickel, platinum, tungsten, molybdenum, tantalum, and alloys of many of these metals have all been successfully used to provide satisfactory recordings. With iron anodes, there is the possibility of a faint reading occurring on the reverse side of the sheet due to the formation of moderately colored oxidation products.

Irrespective of the manner in which the recording sheet is prepared, or the type of electrode utilized, the synchronization of paper feed and current flow with the facsimile signals causes dye to be formed only at points corresponding to gray, colored or black points on the original subject-matter transmitted, thus producing a facsimile recording. Half-tones are obtained because the intensity of color is a function of the amount of dye formed, which increases with increase of current strength, dependent upon electric impulses emanating from the source of transmission. After recording has been accomplished, the paper is exposed to strong light in order to destroy the unchanged diazonium salt, and thus fix the white background. The recordings may also be washed, thereby removing the unused chemicals, as most of these dyes are fast to washing.

While the invention has been described in accordance with illustrative embodiments, it is apparent that many variations and modifications both as to procedural details, steps, and composition may be made without departing from the scope of equivalents within the purview and spirit of the invention as defined in the claims.

The term "facsimile" as used herein is intended to involve not only the reproduction on the recording material of a pre-existing subject, for example, a photograph which is scanned and reproduced in accordance with the impulses ema-

nating from the scanning operation, but also embraces the recording of subject matter in the process of creation or formation without a physically pre-existing subject. As illustrative of this latter category would be the recording of simply a mental preconception, for example, a pattern or design, either of a single color and shades thereof, or multicolors, which is recorded in accordance with an appropriate manual or automatic variation of the electric impulses delivered to the electrodes. Similarly in this category is intended the recording of an arbitrary or hazard design, pattern or other subject, for example, one secured by haphazardly or arbitrarily varying electric impulses delivered to the electrode by punching keys on a master keyboard having suitable electrical connections, by manually or automatically varying resistance, or the like.

Having thus described the invention, what is claimed as new and desired to be secured by Letters Patent is:

1. A fibrous sheet material for the electrolytic formation of azo dye image records thereon treated with an aqueous solution consisting substantially of a dye-forming composition comprising as the aromatic diazonium compound a diazotized para-diaminobenzene in which one amino group is alkylamino, a sufficient quantity of a water-soluble inorganic salt as the electrolyte to facilitate the passage of the electrolyzing current, a sufficient quantity of an azo dye coupling component to react with said diazonium compound to produce an azo dye, and a sufficient quantity of a reducing agent to minimize any air oxidation of said composition to thereby insure a light background for the dye image records, said composition being acidic in nature to preclude premature coupling of said diazonium compound and said azo dye coupling component.

2. The fibrous sheet material as defined in claim 1 wherein the reducing agent is tartaric acid.

3. The fibrous sheet material as defined in claim 1 wherein the aromatic diazonium compound is a mixture of diazotized p-aminodienylaniline and diazotized p-aminodimethylaniline.

4. The fibrous sheet material as defined in

claim 1 wherein the aromatic diazonium compound is a mixture of diazotized p-aminodienylaniline and diazotized p-aminodimethylaniline and wherein the coupling component is a mixture of phloroglucinol and Chicago acid.

NELLIE W. SOLOMON,  
*Administratrix of Estate of Myer Solomon, deceased.*

## REFERENCES CITED

The following references are of record in the file of this patent:

## UNITED STATES PATENTS

| 15 | Number    | Name             | Date           |
|----|-----------|------------------|----------------|
|    | 168,466   | Edison           | Oct. 5, 1875   |
|    | 761,130   | Loeb             | May 31, 1904   |
|    | 1,844,199 | Bicknell et al.  | Feb. 9, 1932   |
|    | 1,880,449 | Hickman et al.   | Oct. 4, 1932   |
| 20 | 1,892,099 | Cornell          | Dec. 27, 1932  |
|    | 1,916,947 | Haendel          | July 4, 1933   |
|    | 1,970,539 | Bausch           | Aug. 21, 1934  |
|    | 2,063,992 | Elsey            | Dec. 15, 1936  |
| 25 | 2,108,852 | Gettinger        | Feb. 22, 1938  |
|    | 2,173,141 | Talmy            | Sept. 19, 1939 |
|    | 2,181,533 | Kline et al.     | Nov. 28, 1939  |
|    | 2,306,471 | Solomon          | Dec. 29, 1942  |
|    | 1,457,581 | Leonardi         | June 5, 1923   |
|    | 1,588,482 | Matthews         | June 15, 1926  |
| 30 | 1,803,532 | Krzikalla et al. | May 5, 1931    |
|    | 2,214,559 | Lecher et al.    | Sept. 10, 1940 |
|    | 2,263,616 | Dahlen et al.    | Nov. 25, 1941  |
|    | 2,154,918 | Schneider et al. | Apr. 18, 1939  |
|    | 2,186,732 | Schneider et al. | Jan. 9, 1940   |
| 35 | 2,186,850 | Wilmanns et al.  | Jan. 9, 1940   |
|    | 2,286,662 | Weyde et al.     | June 16, 1942  |
|    | 2,309,492 | Albers et al.    | Jan. 26, 1943  |
|    | 1,965,635 | Flett            | July 10, 1934  |

## FOREIGN PATENTS

| 40 | Number | Country | Date        |
|----|--------|---------|-------------|
|    | 81,241 | Germany | May 7, 1895 |
|    | 86,828 | Germany | May 6, 1896 |

## OTHER REFERENCES

Color Index, pages 201 and 202, by F. W. Rowe, Jan. 1924.

The Aromatic Diazo, Compounds and Their Technical Applications, by K. H. Saunders, 1936, London, Edward Arnold and Co., pages 30, 36.